

June 9, 1942.

F. W. DUNMORE

2,285,421

HUMIDITY VARIABLE RESISTANCE

Filed June 8, 1940

2 Sheets-Sheet 1

Fig. 1.



Fig. 1a.



Fig. 2.



Fig. 5.



Fig. 3.

Fig. 6.

Francis W. Dunmore,

INVENTOR

BY *J. M. Matherhead*

ATTORNEY

June 9, 1942.

F. W. DUNMORE

2,285,421

HUMIDITY VARIABLE RESISTANCE

Filed June 8, 1940

2 Sheets-Sheet 2



Fig. 4.



Fig. 8.



Fig. 7.



Fig. 8a.



Fig. 9.



Fig. 10.



Fig. 11.



Fig. 12.



Fig. 13.

Francis W. Dunmore,

INVENTOR

BY *J. G. Mathershead*

ATTORNEY

Fig. 14.

## UNITED STATES PATENT OFFICE

2,285,421

## HUMIDITY VARIABLE RESISTANCE

Francis W. Dunmore, Washington, D. C., assignor  
to Government of the United States, as repre-  
sented by the Secretary of Commerce, and his  
successors in office

Application June 8, 1940, Serial No. 339,530

16 Claims. (Cl. 177—351)

(Granted under the act of March 3, 1883, as  
amended April 30, 1928; 370 O. G. 757)

The invention herein disclosed may be used by or for the Government of the United States for governmental purposes without the payment of any royalty therefor.

The wet and dry bulb method of measuring humidity has long been a common means of determining the moisture content of air. There are, however, many circumstances in which this method is not applicable, a particular case being the measurement of upper-air humidities by means of the radio sonde. In fact in all cases where humidity readings are to be read remote from the point of measurement, recorded graphically, or where measurements must be made in small confined spaces or at low temperatures, the wet and dry bulb method is not practical. Attempts have been made to use the hair-type hygrometer but its slow rate of response and other peculiarities have made its use undesirable in many incidences. In radio meteorography the large time lag in response of the hair hygrometer introduces serious errors, since sudden humidity changes are often encountered by a rapidly ascending balloon. This lag increases with decreasing temperature so the accuracy of this type of hygrometer becomes progressively less with increasing altitude.

In my earlier application, Ser. No. 247,243, filed December 22, 1938, an electrical type of hygrometer is disclosed which is particularly adapted for use with the radio sonde, and which, used with certain precautions, more nearly satisfies all the requirements for a remote humidity indicating device without moving parts or appreciable lag. The form therein disclosed consisted of two fine tinned copper wires spirally wound simultaneously on a thin-walled etched glass tube so as to form 20 dual turns per inch. After winding, the glass tube was preferably coated with a dilute solution of lithium chloride in water. The lithium with the moisture which it takes up from the air formed a resistor on the glass surface between the two wires which varied greatly with the moisture content of the air so that the resistance of the unit could be expressed in terms of percent relative humidity. Such a unit gave satisfactory results when certain precautions were observed in its use. These precautions were necessary because of a continuous short and long period aging effect, and a polarization error when used in direct-current circuits. It was also found necessary to switch in two or more units of different sensitivity in order to cover the full humidity scale.

The present invention relates to such an elec-

trical hygrometer and aims generally to improve the same. This invention aims in particular to overcome the above mentioned difficulties, severally, and collectively, and to produce a unit particularly, but not exclusively, suitable for radio sonde use, and which also has advantages over the wet and dry bulb method under many other conditions of measurement. It makes possible more reliable humidity readings, graphically recorded if desired, remote from the point of measurements, as well as more accurate measurements in confined and inaccessible spaces. The original features of rapid rate of response and inherent variation in resistance with humidity have been retained.

In the accompanying drawings illustrative of the improvements of the present invention—

Figs. 1 and 1a are side and end elevations, respectively, of a unit embodying features of the invention;

Figs. 2 and 3 are diagrammatic showings of preferred multiple unit arrangements according to the invention;

Fig. 4 is a diagram showing one form of connection for alternately transmitting humidity and temperature indicating factors;

Fig. 5 is a representative graph for evaluating true humidity from observed humidity and temperature;

Fig. 6 is a graph illustrating frequency-observed humidity characteristics of the arrangement of Fig. 3;

Fig. 7 is a comparative flight record of humidity and temperature plotted against altitude, showing in solid lines the rapid response of the device of the present invention as compared with the response of a concurrently used hair hygrometer, shown in dotted lines.

Fig. 8 is a further chart showing relative speed of response of a hair hygrometer (dotted line) and an electric hygrometer according to this invention (solid line) at 0° C. when taken from air at 30% relative humidity and put in a 500 ft. per minute air stream at 66% relative hu-

midity.

Fig. 8a is a similar chart showing relative speed of a hair hygrometer (dotted line) and an electric hygrometer according to this invention (solid line) at 24° C. when taken from air at 68% relative humidity and put in a 500 ft. per minute air stream at 35% relative humidity.

Fig. 9 shows diagrammatically a preferred arrangement for alternating current operation of the device.

Fig. 10 is a humidity-resistance graph for five

individual units A, B, C, D and E, at 24° C., coated with 6:1 polyvinyl acetate containing 0%; 0.25%; 0.5%; 1.0% and 2.2% lithium chloride solution, respectively.

Fig. 11 is a humidity-resistance graph at 24° C. of the five element electric hygrometer circuit of Fig. 2, with R<sup>1</sup>, R<sup>2</sup>, R<sup>3</sup>, R<sup>4</sup> and R<sup>5</sup> valued at 0.075, 0.15, 0.35, 1.0 and 3.0 megohms respectively; and with units A, B, C, D and E having the same values as in Fig. 10.

Fig. 12 illustrates a multi-scale arrangement for the indicating meter enabling direct reading of relative humidity corrected for any temperature between +30 and -30° C..

Fig. 13 shows a multi-scale arrangement for use at room temperature, using five electric hygrometer units (which may be valued as in Fig. 10 and connected as in Fig. 9) each covering a different part of the humidity range, and

Fig. 14 is a block diagram of an oscillator powered portable device embodying features of this invention.

Certain of what are now regarded as the more important improvements affected by various features of the present invention may be classified under five headings: (1) prevention of long-period aging; (2) prevention of a hysteresis effect or short-period aging; (3) discovery of the advantages of using partially hydrolyzed polyvinyl acetate film, (a) as a binder for hygroscopic salt, (b) in producing a homogeneous film; (c) for reduction of polarization; (4) improved structure and methods of obtaining same; and, (5) special provisions for covering the full humidity range preferably without switching means.

#### 1. PREVENTING LONG-PERIOD AGING

Research work with the dual-coil electric hygrometer described in my above identified application has shown that the electrical resistance of the unit therein described continued to increase from week to week so that it was necessary to calibrate the device shortly before using. It has since been found that this increase in resistance was due to some form of film which gradually formed on the surface of the wire used for the dual coil. After winding units with many kinds of wire, it has now been discovered that this aging effect can be eliminated by employing platinum or palladium wire. As palladium is cheaper than platinum the former is preferred. Twenty dual turns per inch of No. 38 American wire gauge appear to give the best results. Any fewer turns per inch increases the current density at the surface of the wire which tends to increase the polarization effect in direct-current circuits as well as to decrease the life of the unit in alternating current circuits.

#### 2. ELIMINATION OF SHORT-PERIOD AGING

Another phenomenon termed hysteresis or short period aging also made it necessary to calibrate the units of my prior application shortly before using, or to store them at a fixed humidity. The cause of this effect has now been discovered to be the adsorption of water by the etched glass surface upon which the dual coils were wound, and to which the lithium chloride coating was applied. As this giving up or taking on of water by the glass required several hours the result was a shift in the calibration curve for the unit to lower values of resistance if the unit had been exposed to a high humidity for several hours or to higher resistance values if the unit had been exposed to a low humidity for several hours.

The only way to overcome this effect in the units described in my previous application was to store the units in a fixed humidity chamber until ready for use.

After an exhaustive study of many water-resistant coatings on the glass, one coating material has now been discovered which overcomes this troublesome effect; namely, polystyrene resin thermoplastic material. This material is sold by the Bakelite Corporation, under the trade designation "XMS10023," and by the Advance Solvents & Chemical Corporation under the trade-name "Resoglaz." A coating of this material is applied to the glass or other supporting surface by dissolving the polystyrene in one of its solvents with some plasticizer and dipping the supporting surface in this solution. Or polystyrene may now be obtained in film form 1 mil. thick which may be wrapped 3 or 4 times around the supporting surface.

The construction now preferred, however, consists of a thin-walled aluminum tube in place of the glass tube. The aluminum tubing is dipped in the polystyrene solution or is wrapped with 4 turns of the polystyrene film and then wound with the bifilar coil or palladium wire. The aluminum tubing is preferably of the commercial hard tempered type with an outside diameter of  $\frac{3}{8}$  inch and a wall thickness of, say 0.01 inch. A thin wall is necessary as the unit must maintain the temperature of the air surrounding it in order to register the true relative humidity. This is especially important in radio sonde use where sharp temperature inversions are often encountered. Such a unit is shown in Figs. 1 and 1a, described hereinafter.

The polystyrene film on the aluminum tube thus serves as a surface of high electric resistance for the bifilar coil and the moisture-sensitive coating, without influencing the functioning of the device.

In applying this film it is important that the polystyrene solution is such that the film will dry without cracking or crazing. Any such surface irregularities tend to produce a hysteresis effect or lag in response of the device. Also such a surface structure causes non-uniformity of the coating of the moisture sensitive film which is applied after the unit is wound. If a polystyrene film is used in sheet form and wrapped around the aluminum tube it is important that this process does not produce cracking or crazing in the film.

A satisfactory polystyrene solution for coating the aluminum tubing by dipping may be made up by dissolving about 4 to 6 parts by weight of polystyrene ("Resoglaz") with about 1 part by weight of plasticizer such as dibutyl phthalate, in a suitable solvent, preferably consisting of about 4 to 6 parts by weight each of xylene and ethyl acetate mixed with about 7 to 8 parts each of toluene and butyl acetate.

A suitable quantity of solution for laboratory use has been made up of:

|                                 | Grams |
|---------------------------------|-------|
| Polystyrene ("Resoglaz")        | 100.0 |
| Dibutyl phthalate (plasticizer) | 18.4  |
| Ethyl acetate                   | 90.0  |
| Butyl acetate                   | 133.0 |
| Xylene                          | 90.6  |
| Toluene                         | 135.0 |

In coating with this solution the aluminum tubing (with ends closed) was dipped in the solution and immediately withdrawn at a steady rate of

approximately 1 inch per 7 seconds. This process was repeated with a drying interval between each coat of 3 hours until the film of styrene resin was 0.01 inch thick. After the last coat the units were heated at 80° C. for 18 hours before winding. The polystyrene surface was not, and should not be roughened as such treatment produces units which are not reproducible when coated with the moisture sensitive film.

3. DISCOVERY OF ADVANTAGES OF USING PARTIALLY HYDROLYZED POLYVINYL ACETATE FILM

a. Use as a binder for the lithium chloride

The moisture-sensitive material used on the polystyrene surface in the lower ranges of humidity comprises a suitable salt solution, preferably a dilute solution of lithium chloride in water. In order to keep the lithium chloride on the smooth polystyrene surface, a suitable binder had to be found for it which would mix readily with the lithium chloride water solution and form a thin film which would readily pass water vapor without producing appreciable lag in the response of the unit.

During the work on the electrical hygrometer search was conducted for various hygroscopic materials and revealed that a polyvinyl acetate called "Hydrogel" or "Solvar" was somewhat hygroscopic. Such material was accordingly tried (without lithium chloride) as a sensitive hygroscopic coating on shellac spar varnish and balata as bases. These combinations were not well suited for radiometeorological use. In connection with the present invention it has been discovered that this material carried by a polystyrene surface, particularly when mixed with lithium chloride, produces a most satisfactory sensitive element. When applied to the polystyrene resin surface the lithium chloride provides the water-vapor sensitive element and the polyvinyl acetate film the hygroscopic binder for the lower ranges of humidity. The material is known as partially hydrolyzed polyvinyl acetate (36% saponifiable). It is sold by the Shawinigan Products Corporation, Empire State Bldg., New York city, under the name of "Solvar"—sample 6341 S. O. 1232, W. O. 5356-11 Reissue Patent #20,430. A proper concentration of this material was determined to be 1 part of it by volume to 6 parts (by volume) of a mixture of equal parts of water and ethyl alcohol. To this 1-to-6 solution the saturated solution of lithium chloride in water (at 21° C.) is added in percentages by volume depending upon the range in the humidity scale to be covered by the unit to be coated. If used frequently, new solutions should be made each month as the evaporation of the alcohol causes the solution to become more concentrated. The percentages deemed particularly desirable are discussed more fully hereinafter.

b. In producing a homogeneous film

Another advantage in the use of the polyvinyl acetate-lithium chloride combination is that the polyvinyl acetate runs evenly on the smooth polystyrene resin surface. Thereby when combined with the lithium chloride it effects uniform distribution thereof, as well. Lithium chloride and water alone form small globules. With the uniform film, units may be duplicated so that they will agree in their humidity indications to within  $\pm 2\%$ . A satisfactory method of coating is to dip the wound units into the polyvinyl acetate-lithium chloride solution and withdraw them at a steady rate of 1 inch in 12 minutes.

c. For reduction of polarization

A third advantage in the use of the polyvinyl acetate film proved to be a reduction of the polarization or counter E. M. F. set up by the direct current flowing through the unit when used with the radio sonde of the type described in Journal of Research, National Bureau of Standards, vol. 20, pages 367-392 (1938) Research Paper R. P. 1082. In normal use alternating current may be applied to the units when making measurements in which case polarization errors are not present. However, it is necessary to use the same type of circuit or indicating instrument as was used in calibrating the units as the resistance of the unit is somewhat a function of the current flowing through it. The unit behaves a little like an electrolyte.

The reason for the reduction of polarization by the polyvinyl acetate film is not fully understood but since the film is more like a solid than a liquid its electrical conduction characteristics are perhaps more like those of a solid.

4. IMPROVED STRUCTURE AND METHODS OF PRODUCING SAME

A typical single unit according to the invention shown in Figs. 1 and 1a may consist of a winding 10 of, say, 32 inches (about 25 bifilar turns) of No. 38 (American wire gauge) bare soft-drawn palladium wire (ultimate tensile strength 600 grams) wound 20 bifilar turns per inch on a polystyrene-coated aluminum tube 11. The tubing may be about 1 $\frac{1}{8}$  inches long with an outside diameter of  $\frac{3}{8}$  inch and a wall thickness of 0.01 inch. The devices may be provided with insulated end washers 12 at one end, serving, as by solder eyelets 14, to hold the terminal leads 15, while the washers 13 at the other end serve to anchor the free ends of the dual coil 10, which in the embodiment shown are twisted about ears 13a formed on washers 13. These washers 12 and 13 are preferably made of polystyrene resin and are preferably applied over the polystyrene resin coat and "anchored," as with a drop or two of the polystyrene solution, about  $\frac{1}{8}$  inch from the ends of the tube 11. This gives a longer leakage path from the terminals to the aluminum tubing. Where sufficient rigidity can be obtained with a unit moulded from polystyrene resin with a wall thickness of 0.02 inch, then this invention contemplates that the whole unit, washers and all, may be moulded in one piece without the need for the aluminum tubing. As high temperatures might cause such a unit to lose shape and thereby loosen the winding, the formation of the device on an aluminum tube is preferred for general use.

In order to insure a tight winding the palladium wires in accordance with this invention are heated as they go on to the tubes so that they seat just slightly into the styrene resin surface.

In order to obtain units with predetermined operating characteristics, it is important that a standard method of applying the polyvinyl-acetate-lithium-chloride coating be followed. A satisfactory procedure is to mount the units with their longest axis vertical. They are quickly immersed up to the terminal washer in the solution and then withdrawn by a motor-driven device at a constant rate of 1 inch in 12 minutes. The surplus liquid clinging to the lower end of the unit is absorbed with a blotter, and the units are allowed to dry in still air.

After the units are coated, they must go through an aging period of at least 10 to 14 days

before they are ready for use. During this time the resistance of the units continues to decrease until it settles down to a final value (for any given humidity) where it remains for many months. Recent experiments on 19 units seem to indicate that this aging period may be reduced to 2 days by putting the units in a humidity chamber with air at 60-percent relative humidity and 26° C. and continually circulating the air gently over the units.

#### 5. SPECIAL PROVISIONS FOR COVERING THE FULL HUMIDITY RANGE WITHOUT SWITCHING MEANS

If an attempt were made to cover the full humidity range with a single unit such as shown in Fig. 1, the variation in resistance of the unit would be so extreme that it would extend outside the normal limits of a measuring device. Furthermore, the excessive current through the unit at high humidities might be harmful to the unit.

In the case of the radio sonde the resistance variation for a change in humidity from 5 to 100% from +30° C. to -30° C. should preferably be kept within the limits of 3 megohms to 10,000 ohms. When used in an A-C. circuit such as with a Weston model 764 microfarad-meter (calibrated to read in ohms) the resistance variation for a change from 5 to 100% humidity should be confined within the limits from 8 megohms to 75,000 ohms.

In order to make possible this condition my invention contemplates the provision of a multiple unit having different percentages of LiCl coatings on each of its elements. Thus by arranging a number of units in parallel, with the proper resistors in series with each, it is possible to confine the resistance variation of the composite unit to the desired limits.

Such an arrangement is shown in Fig. 2, a five unit embodiment, in which unit A may have a polyvinyl-acetate coating only; unit B, a coating of 0.1% LiCl; C, 0.5% LiCl; D, 1.0% LiCl; E, 2.0% LiCl. Resistance  $R_5$  in this embodiment is greater than  $R_4$ ; resistance  $R_4$  is greater than  $R_3$ , etc. At the high humidities units B, C, D and E, although practically shorted, are prevented from causing a short at terminals F by resistors  $R_2$ ,  $R_3$ ,  $R_4$  and  $R_5$  yet the resultant resistance at E will vary below the values of  $R_2$ ,  $R_3$ ,  $R_4$  and  $R_5$  since unit A has resistor  $R_1$  only in series with it. Thus A is the controlling unit at high humidities. On the other hand, at low humidities A, B, C and D are practically open-circuited while  $R_1$ ,  $R_2$ ,  $R_3$ ,  $R_4$  and  $R_5$  are not sufficiently high to prevent the change in resistance of unit D from effecting the overall resistance at F. Thus E is the controlling unit at low humidities. In a like manner units B, C and D become the controlling unit in turn at intermediate humidities. These operating characteristics are explained more fully hereinafter.

#### OPERATING CHARACTERISTICS IN DIRECT CURRENT RADIO-SONDE CIRCUITS

As the radio-sonde circuits pass pulsating direct current through the electric hygrometer, the characteristics of the unit in such a circuit differ somewhat from those obtained when it is used in alternating current circuits. Some polarization exists in direct current circuits, but it is a fixed factor in a given type of circuit and does not change the calibration of the unit appreciably during the period of a flight (about 1 hour). The unit appears to have a higher resistance at a given humidity than if measured with alternat-

ing current flowing through it as described hereinafter.

#### 1. THREE-ELEMENT UNIT

For use in the radio-sonde circuit developed at the Bureau of Standards (see J. Research N. B. S. vol. 20, R. P. 1082), a three-element unit has been found satisfactory. This unit, illustrated in Fig. 3, consists of three elements constructed as outlined above. The elements are coated with a 1%, 2% and 3% lithium chloride-polyvinyl acetate solution respectively. The three-elements are connected in parallel with 32,500 ohms in series with the 2% and 3% units, and an additional 32,500-ohm resistor in series with the 3% unit.

In radiometeorograph work, the electric hygrometer and an electrolytic thermometer are alternately connected to the radio-sonde circuit in any suitable way. Desirably, this may be effected by means of a single-pole, double-throw relay which is operated in any suitable manner, as by an atmospheric pressure operated switch, traveling across a multi-segment commutator, as shown in Fig. 4, in which the expandable bellows or "Sylphon" 19 moves switch 20 across conducting and non-conducting segments of commutator 21, making and breaking the circuit of relay switch 22 and battery 23. When the relay circuit is open the multi-unit humidity responsive system 24 is connected in the control circuit of frequency generator 25; and when the relay circuit is closed the temperature element 26 is substituted to provide the temperature factor for evaluation of relative humidity.

#### 2. FREQUENCY-HUMIDITY CHARACTERISTIC

In the radio-sonde circuit, the variation in resistance of the electrical hygrometer alters the audio-frequency generated by a relaxation oscillator which in turn modulates the carrier-frequency oscillator. In Fig. 6 is shown the humidity-frequency graphs at 25° C. for the individual 1, 2, and 3% LiCl units when used separately in the radio-sonde circuit. The dotted graph in this figure is for the composite arrangement at 25° C. shown in Fig. 3.

#### 3. TEMPERATURE CORRECTION

The electric hygrometer functions like an electrolyte in that its resistance increases with a decrease in temperature. In radio-sonde use where temperature variations of 100° are encountered it is of course necessary to apply a correction to obtain the true humidity. It has not been found possible, even with a composite 3-element unit, to cover the full 10-100% humidity scale, over this extreme temperature range, but it has been feasible, with the composite unit shown in Figs. 3 and 5 to cover a considerable portion of this range. The family of graphs for different temperatures exemplified in Fig. 5 constitute the standard as determined from the average of many composite units having individual units with characteristic at 25° C. as shown in Fig. 6.

Knowing the temperature (as is the case with a radio sonde) the humidity is obtained from the frequency-humidity graph for that temperature.

If the method previously outlined for making and coating the units is carefully followed, it is

possible to obtain 75-80% of the units which will fall within  $\pm 2$  or 3% of the standard graph.

For use at varying temperatures other than with the radio sonde, a multi-scale indicating instrument may be used as described in connection with Figs. 12 and 13.

## 4. FLIGHT RECORDS

In Fig. 7 there is shown a comparative flight record illustrating the great increase in sensitivity effected by the present invention, as compared to the old style hair-hygrometer. This record shows the two hygrometer traces (solid, electrolytic; dotted, hair) starting at the same point (about 88% relative humidity), and shows clearly the rapid response and very informative reversals detected by the electrolytic hygrometer, which, except in the case of a prolonged reversal, escape the hair hygrometer. The other half of the chart shows the temperature existing at the respective altitudes (see Fig. 4) from which the corrected values of relative humidity may be obtained as discussed in connection with Fig. 5. In this chart the abscissa values are determined by the audio frequency in terms of which the humidity and temperature are transmitted from the radio sonde. The ordinate represents altitude, each changeover from temperature to humidity being made by the atmospheric pressure operated switch at a predetermined pressure which may be converted into altitude in feet.

The records shown in Figs. 8 and 8a, further illustrate the very rapid rate of response of the electric hygrometer to sudden humidity changes. Fig. 8 shows the relative speed of response of the electrolytic hygrometer (solid line) and a hair hygrometer (dotted line) at 0° C. when taken from air at 30% relative humidity and placed in at 500 ft. per minute air stream at 66% relative humidity. Both units it will be seen, start with an observed or indicated value or 30% or 36% less than the 66% terminal value. As shown by the curves, the standard time constant  $P$  of the electrolytic hygrometer (eleven seconds) is twenty times as fast as that of the hair hygrometer  $Q$ , three and one-fourth minutes. The time constant is the time required for the unit to reach a value indication equal to the product of the original difference, here 36%, multiplied by the factor: one minus the reciprocal of  $e$ , the base of natural logarithms, which factor has the value 0.63, placing the time constant line  $PQ$  at the value

$$36-0.63(36)$$

or 36-22.68

which equals 13.32 as shown

Similarly, Fig. 8a shows the relative speed of response of the electrolytic unit (solid line) and a hair hygrometer (dotted line) at 24° C. when taken from air at 68% humidity and put in a 500 ft. per minute air stream at 35% humidity, and shows the time constant  $R$  for the electrolytic unit, 3 seconds, as against 1 minute for the time constant,  $S$ , for the hair hygrometer, in the formula where  $\delta = 68-35$ , or 33 and hence the value for  $RS$  equals  $33-0.63(33)$ , or 12.21, as shown.

It is thus clear that the same 20-to-one improvement pertains both as regards indication of increasing and decreasing humidity.

OPERATING CHARACTERISTICS IN A.-C. 65  
MEASURING CIRCUITS

## 1. CIRCUIT ARRANGEMENT

For use other than with the radio sonde the electrical hygrometer should preferably be used in an alternating current circuit as polarization is thereby eliminated. In the case of the radio sonde this is not a serious factor as it does not alter the operation of the hygrometer sufficiently to change the calibration during the period of

time (say 1 hour) in which the unit is used. A preferred alternating-current circuit arrangement is that shown in Fig. 9. Here the unit 29 is put across about 100 volts 60 cycles alternating current supplied by the adjustable transformer 30, with 766,000 ohms series resistance 31 and the input of a full-wave oxide rectifier 32 in series with it. The direct-current output of the rectifier is connected to a 0-125 microammeter MA. The microammeter scale may be calibrated in terms of percent relative humidity. The voltage impressed on this circuit arrangement should of course be kept at 100, for which purpose any suitable voltage regulator may be used.

The above circuit arrangement is that obtained when using the C/1,000 scale of a Weston model 764 capacity meter, the electric hygrometer taking the place of the condenser to be measured. This capacity meter may be used as an ohmmeter in this fashion, since it is measuring only ohmic resistance in a nonreactive circuit. This circuit arrangement was adopted because it passes alternating current through the unit, and this current is never greater than 200 microamperes. The current must be kept under this value, as heavy currents would alter the calibration. Information as to the constancy of calibration of a unit if the current is allowed to flow through it continuously is not yet available, although a current of 100 microamperes flowing through a unit steadily for several days seemed to have little effect. It is safer, until further data are available, to read humidity by allowing current to flow through the unit only for the time necessary to take a reading, or for control purposes a timing switch may connect the unit into circuit only for a time long enough to affect the control mechanism. If this is not feasible, the hygrometer unit may be left in the control circuit continually by placing it in the input circuit of a suitable electron-tube amplifier with the indicating or control device in the output circuit. In such a circuit the current through the unit will be kept within safe limits.

The capacity between the two wires running to the humidity unit should be kept as small as possible by separating them. If appreciable, a circuit arrangement described hereinafter may be used.

## 2. HUMIDITY-RESISTANCE CHARACTERISTICS

## a. Single-unit characteristics

Using such a circuit arrangement with the capacity meter calibrated to read in ohms instead of microfarads, the humidity-resistance characteristics shown in Fig. 10 were obtained. Here graphs B to E are for standard units with a 0.25-, 0.5-, 1-, and 2.2-percent LiCl coating, respectively. Graph A is that obtained with the polyvinyl-acetate film alone, without LiCl.

The coatings on these units were so chosen that each unit covers a different range of humidity when varying over the same resistance. Thus, considering a resistance variation from 8 megohms to 75,000 ohms, unit E covers from 10 to 22 percent, unit D 22 to 42 percent, unit C 40 to 60 percent, unit B 50 to 70 percent, unit A 66 to 91 percent. A percentage of LiCl for B to give less overlap would be 0.10 percent, and in this case A may be coated with a somewhat diluted polyvinyl-acetate solution, to cause the unit to register up to 100 percent.

## b. Composite-unit arrangement

While individual units as described above

should find some applications as described hereinafter. It is evident from Fig. 10 that no one unit will cover the full humidity scale. However, by putting the units A to E (Fig. 10) in parallel each with its proper series resistor, as shown in Fig. 2, it is possible to obtain in effect a single unit which covers the humidity range from 10 to 100 percent at room temperatures, with resistance variation confined within the limits of 8 megohms to 75,000 ohms. A satisfactory combination from Fig. 3 is:  $R_1=75,000$  ohms,  $R_2=0.15$  megohms,  $R_3=0.35$  megohm,  $R_4=1$  megohm,  $R_5=3$  megohms, with A coated with polyvinyl acetate only, B with 0.25 percent of LiCl, C with 0.5 percent of LiCl, D with 1 percent of LiCl, and E with 2.2 percent of LiCl. The resistances required will vary somewhat with the variation in the range of response of different units with the same percentage of coating. The humidity-resistance graph for the above combination is shown in Fig. 11. With such an arrangement the microammeter scale may be calibrated to read in terms of relative humidity instead of ohms. Such a composite unit has not varied over 3 percent from an original calibration, over a period of 4 months.

#### DESIGNS FOR SPECIAL USES

A hygrometer of the type described is very flexible in its application, since it is of the electrically operated type and may be modified to fit specific needs.

If one is interested in a limited humidity range, as for example in the automatic control of humidity, a single-element unit is desirable, as greater sensitivity may be obtained. (See graphs in Fig. 10.) It must be emphasized, however, that information is not yet available as to the life of a unit when the control current is allowed to flow through it continually. An electron-tube amplifier or a timing switch may be used, as described above. Replacement units are inexpensive and may be easily plugged into circuit after a given number of hours.

##### 1. DESIGN FOR USE WHERE A.-C. POWER IS AVAILABLE

Where it is necessary to run long lines from the humidity-indicating device to the humidity unit, it is desirable to locate the full-wave oxide rectifier 32, as shown in Fig. 9, at the location of the humidity unit and run the direct current output of the rectifier back to the location where the humidity is to be registered. This method is preferred, as the alternating current flowing across the capacity of a long line to the humidity unit would register on the indicating meter.

##### 2. BATTERY-OPERATED UNIT

For portable use and in places remote from a 60-cycle alternating current supply a measuring circuit may be used in which the alternating current for operating the unit is obtained from an electron-tube oscillator operating at 60 cycles. It may be powered from small dry cells such as are used in portable radio sets. Such an arrangement is shown in Fig. 14, in which the alternating current is supplied through the unit 33 by oscillator 34 to the input terminals 35 of amplifier unit 36, the output terminals 37 of which are connected to the indicating instrument 38 of conventional design.

##### 3. MULTISCALE UNIT FOR CONDITIONS OF WIDE TEMPERATURE VARIATIONS

For registering humidity under a condition of wide variation in temperature, a multiscale in-

dicator such as shown in Fig. 12 may be used. Knowing the temperature, the humidity scale for that temperature is used.

A second type of multiscale arrangement for use at room temperature is shown in Fig. 13. Here individual units with different sensitivities are connected to the measuring instrument (Weston model 764 capacity meter set at minimum capacity setting) by means of a five-point switch. Depending upon the humidity, the particular unit may be selected which brings the meter reading within the scale. Thus if the humidity is between 10 and 20 percent, switch contact 1 and scale 1 will be used. This arrangement has the advantage of very open scale, allowing greater precision in humidity headings.

Various details of the present invention are described in an article by the present inventor, to which reference is hereby made, entitled "An improved electric hygrometer," published as research paper R. P. 1265, in the Journal of Research of the National Bureau of Standards, vol. 23, No. 6, Dec. 1939, page 701, et seq., and to which reference may be had to supplement the foregoing description if desired.

From the foregoing description it will be appreciated that various modifications may be made without departing from the invention exemplified in the preferred embodiments disclosed.

Thus, while polystyrene, polyvinyl-acetate and lithium chloride are preferred constituents found particularly desirable in embodying this invention, in its broader aspects the invention is not limited to the use of these materials.

I claim as my invention:

1. A humidity variable device comprising a support of high electrical resistance non-hygrosopic material, bifilar conductors carried thereby, and a thin film of intermixed hygroscopic and binder materials in electrical contact with and overlying said bifilar conductors.

2. A humidity variable device comprising a support of high electrical resistance non-hygrosopic material, bifilar conductors carried thereby, and a film of hygroscopically sensitized polyvinyl acetate in electrical contact with said bifilar conductors.

3. A humidity variable device comprising a support of high electrical resistance non-hygrosopic material, bifilar conductors carried thereby, and a film of polyvinyl acetate hygroscopically sensitized with lithium chloride embedding said bifilar conductors.

4. A humidity variable device comprising a thin highly heat conductive base, a support of high electrical resistance non-hygrosopic material carried by said base, bifilar conductors carried by said support, and a thin hygroscopically sensitive film in electrical contact with and overlying said bifilar conductors.

5. A humidity variable device comprising a thin-walled aluminum tube, a thin layer of non-hygrosopic electrical insulating material thereon, bifilar conductors wrapped on said insulating material, and a thin hygroscopically sensitive film in electrical contact with and overlying said bifilar conductors.

6. A humidity variable device comprising a thin highly heat conductive base, a thin supporting layer of polystyrene resin thereon, bifilar conductors supported by said layer, and a hygroscopically sensitive film in electrical contact with said bifilar conductors.

7. A humidity variable device comprising a thin aluminum base, a thin supporting layer of

polystyrene resin thereon, bifilar conductors supported by said layer, and a hygroscopically sensitive film in electrical contact with said bifilar conductors.

8. A humidity variable device comprising a thin walled aluminum tube, a supporting layer of polystyrene adhering to said tube, bifilar conductors wrapped on said polystyrene and slightly seated therein, and a film of polyvinyl acetate hygroscopically sensitized with lithium chloride adhering to said conductors and said polystyrene support.

9. In a humidity variable device of the type described, a non-hygroscopic polystyrene support, bifilar conductors carried thereby, and a hygroscopically sensitive film in electrical contact with said conductors.

10. In a humidity variable device of the class described, a thin aluminum base having a non-hygroscopic polystyrene resin coating thereon, bifilar conductors seated slightly in said polystyrene resin, and a hygroscopically sensitive film overlying said conductors and said polystyrene coating and in electrical contact with said conductors.

11. In an electrical hygrometer circuit, a humidity responsive element comprising bifilar conductors electrically connected by a hygroscopically sensitive film, a source of predetermined alternating current, a rectifier, a circuit connecting said current source and said element with the input of said rectifier to supply thereto an alternating current controlled by said element, and means for measuring the direct-current output of said rectifier as a measure of the humidity-indication of said element.

12. A humidity responsive system comprising an electron tube generator of alternating current, an electron tube amplifier, a humidity responsive element comprising a supporting area of high electrical resistance non-hygroscopic material, bifilar conductors carried by said area and a hygroscopically sensitive film in electrical contact with said bifilar conductor, a control circuit for said amplifier powered by the output of said generator, said humidity responsive element being connected in said control circuit, and translating means operated by the output of said amplifier.

13. A humidity variable device comprising a support of high electrical resistance non-hygroscopic material, a pair of spaced conductors carried thereby and a thin film of intermixed hygroscopic material and amorphous material pervious to moisture in electrical contact with and overlying said pair of conductors.

14. In a humidity device having two electrical terminals; a plurality of elements; each element comprising a supporting area of highly non-hy-

groscopic material having a high electrical resistance, two separated electrical conductors carried by said area, and a hygroscopically sensitive film in contact with said conductors and said supporting area; the hygroscopic films on said respective elements containing binder material and hygroscopic salt in different proportions, respectively; said device further comprising electrical resistors of different values and having one conductor of each element connected to one of its said electrical terminals and the other conductor of each element connected through one or more of said resistors of different value to the other of its said electrical terminals, and having the values of resistance in series with its respective elements greater, the greater the amount of hygroscopic salt in the film of the respective element.

15. In a humidity device having two electrical terminals; a plurality of elements; each element comprising a supporting area of highly non-hygroscopic material having a high electrical resistance, two separated electrical conductors carried by said area, and a hygroscopically sensitive film in contact with said conductors and said supporting area; the hygroscopic films on said respective elements containing binder material and hygroscopic salt in different proportions, respectively; said device further comprising an electrical resistor and having one conductor of each element connected to one of its said electrical terminals, the other conductor of one of its elements connected to the second of its said electrical terminals, and the other conductor of another of its elements connected through said resistor to the second of its said electrical terminals.

16. In a humidity device having two electrical terminals; a plurality of elements; each element comprising a supporting area of highly non-hygroscopic material having a high electrical resistance, two separated electrical conductors carried by said area, and a hygroscopically sensitive film in contact with said conductors and said supporting area; the hygroscopic films on said respective elements containing a hygroscopic binder fortified, save for one element, with different amounts of hygroscopic salt; said device further comprising electrical resistors of different values and having one conductor of each element connected to one of its said electrical terminals and the other conductor of each element connected through one or more of said resistors of different value to the other of its said electrical terminals, and having the values of resistance in series with its respective elements greater, the greater the amount of hygroscopic salt in the film of the respective element.

FRANCIS W. DUNMORE.